

## UNITED STATES PATENT OFFICE

LÉON LOUIS MATHIEU, OF ROUEN, FRANCE, ASSIGNOR TO SOCIETE ANONYME DES HAUTS-FOURNEAUX ET FONDERIES DE PONT-A-MOUSSON, OF PONT-A-MOUSSON, MEURTHE-ET-MOSELLE, FRANCE

## MOLDING SAND

No Drawing. Application filed December 29, 1928, Serial No. 329,204, and in France April 27, 1928.

This invention relates to a composite sand or molding material especially adapted for use in casting pipes by the centrifugal method and comprising sand together with a certain amount of coal tar, the amount of coal tar being preferably about 1 or 2 per cent by volume.

The proportions in the composition may be, for instance, as follows:

|                | Parts by volume |
|----------------|-----------------|
| Siliceous sand | 40              |
| Old sand       | 20              |
| Clayey sand    | 13              |
| 15 Coal tar    | 1               |

The improved molding material offers great advantages, chiefly when the pipes are cast by the centrifugal process in a sand mold contained in a metal mold made in one piece. In such a case, not only the amount of sand required should be reduced to a minimum but also the sand should allow the metal to be cast without any preliminary drying of the sand. The sand must also be used without any coating adapted to prevent its adhesion to the cast metal, and the pipe should be readily removable from the mold after the casting. This latter operation is made more difficult due to the fact that the pipe usually has a raised edge or annular bead which tends to prevent the removal of the cast pipe from the mold.

The composite sand or molding material according to the invention answers the above requirements. It possesses a great cohesion and provides for casting operations without preliminary drying and without any preliminary coating of an expensive nature.

40 During the casting operation, there is produced a distillation of the tar, thus automatically covering the mold with a layer protecting it against the cast metal. After the casting, the tar is burnt away, whereby the sand 45 is disaggregated, so that it will not materially oppose the discharge of the pipe and the exit of its said raised edge.

Obviously, the above mentioned composition of the sand is given solely by way of example. The proportion of tar employed

will depend upon the dimensions of the pipes or like pieces to be cast.

Having now described my invention what I claim as new and desire to secure by Letters Patent is:

A molding material comprising the following substances:

|                | Parts by volume |
|----------------|-----------------|
| Siliceous sand | About 40        |
| Old sand       | About 20        |
| Clayey sand    | About 13        |
| Coal tar       | About 1         |

In testimony whereof I have signed my name to this specification.

LEON LOUIS MATHIEU.

55

60

65

70

75

80

85

90

95

100